

Dec. 9, 1930.

W. R. WHITNEY

1,784,647

METHOD OF MAKING CRUCIBLES

Filed Nov. 3, 1926

Fig. 1.



Fig. 2.



Inventor:  
W. R. Whitney

## UNITED STATES PATENT OFFICE

WILLIS R. WHITNEY, OF NISKAYUNA, NEW YORK, ASSIGNOR TO GENERAL ELECTRIC COMPANY, A CORPORATION OF NEW YORK

## METHOD OF MAKING CRUCIBLES

Application filed November 3, 1926. Serial No. 146,047.

My invention relates to crucibles and more particularly to crucibles for electric induction furnaces, and has for its object the production of a simple and rugged crucible having a heating resistor incorporated in its walls.

My invention has particular application to the making of crucibles used with high frequency electric induction furnaces in which a material having high electrical resistance, such as carbon or graphite, is embedded in the wall of the crucible to form a heating resistor, electric currents being produced in it by electrical induction.

5 In carrying out my invention in one form, I construct the crucible from a suitable heat refractory material which may be molded in plastic form, such as fire clay, with which is mixed a suitable amount of carbon or graphite 10 to form a heating resistor. After being molded the crucible is suitably fired in a reducing atmosphere and then finally heated in the open air to a temperature sufficient to burn out the carbon or graphite from an outer layer 15 of heat refractory material. This produces a crucible of unitary structure which is provided with an inner embedded heating resistor covered with an outer layer of fire clay forming a lining.

20 For a more complete understanding of my invention reference should be had to the accompanying drawing in which Fig. 1 is a view partially in section of a crucible embodying my invention, while Fig. 2 is a diagrammatic view illustrating the use of the crucible in a high frequency furnace.

25 Referring to the drawing, the crucible in finished form, as constructed in accordance with my invention, comprises a unitary molded mass of suitable heat refractory material which is provided with an inner portion 10 containing a suitable quantity of high resistance but conductive material sufficient to form an electric resistor, this resistor being 30 covered with an outer layer 11 consisting of the heat refractory material alone. Ordinarily, crucibles of this type are formed by covering a graphite crucible corresponding to the resistor 10 with a layer of heat refractory 35 material.

In accordance with my invention, the crucible is molded or otherwise formed as a unit. In making the crucible, a suitable amount of high resistance material, such as carbon or graphite, is mixed with the plastic heat refractory material, such as fire clay, the resistance material contained being sufficient to give the desired electric resistor heating properties. After the crucible has been molded to the desired shape in any suitable manner, it is fired in a reducing atmosphere, for example, in a porcelain kiln filled with suitable reducing gas, such as hydrogen. After being fired the crucible is finally heated in the open air so as to burn out the resistance material from an outer layer. This results in an outer layer or lining 11 of fire clay, from which the graphite has been burned, with an inner layer of a mixture of fire clay and graphite forming a resistor.

40 In using the crucible in a high frequency furnace, for example, the crucible is inserted in a suitable induction coil 12, Fig. 2, which is supplied with a suitable high frequency current whereby electric heating currents are 45 induced in the inner resistor 10.

50 It will be noted that the crucible is very simple in construction, and furthermore very rugged since there is no danger of the lining becoming loose and detached as often happens when the lining is applied separately.

55 What I claim as new and desire to secure by Letters Patent of the United States is:—

1. The method of making a crucible having an inner heating resistor and an outer heat refractory lining which consists in molding the crucible from a mixture of heat refractory material and powdered resistance heating material, and then burning the resistance heating material out of an outer layer of the heat refractory material so as 60 to leave an inner heating resistor.

65 2. The method of making a crucible having an inner heat resistor and an outer fire clay lining which consists in molding the crucible from the mixture of fire clay and graphite and then burning the graphite out of an outer layer of the fire clay so as to leave 70 an inner heating resistor.

75 3. The method of making a crucible hav-

55

60

65

70

75

80

85

90

95

100

ing an inner heating resistor and an outer heat refractory lining which consists in molding the crucible from a mixture of heat refractory material and powdered resistance heating material, heating said crucible in a reducing atmosphere and then heating said crucible in an atmosphere of air so as to burn the resistance material out of an outer layer of the heat refractory material.

4. The method of making a crucible having an inner heating resistor and an outer fire clay lining which consists in molding the crucible from a mixture of fire clay and graphite, firing said crucible in a reducing atmosphere and then heating said crucible in an atmosphere of air so as to burn the graphite out of the outer layer of the fire clay.

In witness whereof, I have hereunto set my hand this 2nd day of November, 1926.

WILLIS R. WHITNEY.

25

30

35

40

45

50

55

60

65